

# UNITED STATES PATENT OFFICE.

FREDERICK W. HOCHSTETTER, OF DAYTON, OHIO, ASSIGNOR OF ONE-HALF TO W. I. OHMER, OF DAYTON, OHIO.

## TRANSLUCENT MEDIUM FOR USE IN PHOTOGRAPHIC ARTS.

1,419,379.

Specification of Letters Patent. Patented June 13, 1922.

No Drawing. Original application filed November 10, 1919, Serial No. 336,898. This application filed May 21, 1921. Serial No. 471,524.

To all whom it may concern:

Be it known that I, FREDERICK W. HOCHSTETTER, a citizen of the United States, residing at Dayton, in the county of Montgomery and State of Ohio, have invented certain new and useful Improvements in Translucent Mediums for Use in Photographic Arts, of which the following is a specification.

The principal object of my invention is to provide a translucent medium for use in the photographic arts in the place of nitro cellulose compounds now generally used. By nitro cellulose compounds I refer to the various translucent and transparent substances used in photographic and similar arts, many forms of which are termed films.

It is the further object of my invention to provide a medium of translucent character which can be used not only for negatives but also for transparencies and diapositives. The range of usefulness of my invention is only limited so far as the photographic art is concerned, by the limits of the art itself. It is applicable to film purposes for both still photography and moving pictures.

It is one of the signal objects of my invention, that the translucent medium becomes an integral portion of the photographic negative or other use to which it may be put, as distinguished from the attempts in the past to use translucent medium on supports which were merely temporary and had to be removed from the remainder of the negative or positive before the operation could be complete. My object is to provide a permanent base of translucent character like the ordinary film, which shall be entirely fire-proof and not inflammable. This is a very material advantage over the present film with its highly inflammable and explosive character incurring great danger in handling, shipping and use, as well as in the course of manufacture.

It is my object to provide, as has not hitherto been provided, a translucent medium which shows no grain whatsoever and is free from any opacity which might detract from the usefulness and beauty of the resulting images, projections or positives.

Furthermore, I have succeeded in thus making such an advance in the art that the result is not only translucent, without grain and not inflammable, but also I have been able to use the ordinary material found on

the market, such as paper of varying characters, of varying methods of manufacture, of varying lengths of fiber or lengths of material which compose the paper and make up its structure. In accomplishing these several objects, I have not affected the rapidity with which positives may be made from the negatives, nor effected the question of projection of images from film in moving pictures where the film is made up of my translucent material.

A further object of my invention is to so provide such translucent medium that no unpleasant refraction would be encountered in the case of projection of moving pictures due to any refractive properties which might either be left in my translucent medium or created by my process of producing it.

I transform my paper that I use for this purpose, which may be of any kind, although I have some preferences which will be stated later, in the following way: I select a drying oil, such as linseed oil. 10 oz. of this oil is heated to 100 degrees F. I then use a substance to give a hard smooth surface to the paper to which dust will not cling. One of the preferred substances is bleached shellac, of which I use 3 oz. I then select a dehydrating agent such as alcohol, of which I use 20 oz. in this combination. It also acts as a solvent for the shellac and a carrier of it to further the combination of it with other elements of the compound and article.

The substances mentioned above are mixed at 100 degrees F. in the order given successively, although the mixing of the ingredients in any particular order is not essential to my invention, but preferable.

The mixture is now ready for application to the paper in the paper's finished state.

The finished paper is heated to about 100 degrees F. by any suitable means, although I prefer a series of hot rollers of the proper temperature over which the paper is passed to give it a suitable temperature, but care must be used not to heat the paper to such a temperature as to injure its color. I prefer to use white paper, although that is not essential. The paper thus heated is then passed through the solution, the formula for which has been given above. The paper passes out on other rollers, and the temperature is gradually decreased until the paper

is returned to its normal temperature, thus allowing the paper to dry. The paper becomes translucent as soon as the solution thoroughly permeates it.

5 In order to protect the translucency of the paper and to prevent it from being injured, I coat the paper with another substance after it has been treated to make it translucent. This compound, with which it 10 is treated, is as follows: I take 15 grams of hard gelatin, melted by heat, and mix it with 1 oz. of linseed oil and an alcoholic solution of chrome alum. I prefer to use, however, a mixture for this purpose of hard gelatin, 15 melted by heat and bichromate of potash without oil. Either of these compounds will treat the paper to preserve its translucency, act like a mordant and act to prevent the formation of an alkali and to prevent the emulsion from frilling or peeling off from the translucent paper when the sensitizing emulsion is applied. The sensitizing emulsion may be applied either before or after the paper has been made translucent.

20 25 I do not desire to confine myself to the particular components of the compounds that I have enumerated above, because equivalent ingredients may be used if they have the properties for the purposes intended. The temperature that I have stated is a preferred temperature, but it should be understood it is not essential that this temperature be exact.

In case the paper is treated without being 30 heated, in a cold solution, then the solution will be composed of the following: A drying oil, such as linseed oil and a dehydrating agent, such as absolute alcohol. The shellac is omitted. I do not prefer this 35 form.

In case it is desired to make the paper translucent during the course of its original manufacture before it is completed, it is possible to readily do this by passing the paper, 40 after it has sufficiently set, but is still in its plastic state, through the solutions mentioned, depending upon whether or not it is desired to treat the paper at its normal temperature or above its normal temperature.

45 50 One of the preferred forms of a medium for treatment to make it translucent is a paper composed of short fiber cotton made up from rags. Ordinarily, it has been thought that the shorter the fiber, the 55 greater the refraction of light, due to the multiplicity of surfaces within the paper. I find, however, in my invention that the

length of the fiber is not of great moment, although the short fibers are preferable. The use of short fibers will make even more 60 perfect the perfection of my translucency.

If it is desired to treat the paper while in its plastic state with the heated solution, it is passed into the heated solution first mentioned and then passed over heated rollers 65 or conveyors into the second solution and then gradually cooled.

If it is desired to treat it while in its plastic state with the cold solution, the heating arrangements are omitted.

70 In the foregoing, I have mentioned paper and paper pulp as a medium to be treated. In the following claims, I have also mentioned paper and paper pulp. In doing so, I have merely used these terms for the purposes of illustration and suggestion, but I do not desire to be confined to this medium alone for making opaque substances translucent.

75 This application is a division of Hoch- 80 stetter application Serial No. 336,898.

Having thus fully described my invention, what I claim as new and desire to secure by Letters Patent, is:

1. A composition of matter for treating 85 paper to render the same translucent comprising a drying oil, a glazing medium and a dehydrating agent only.

2. In combination, linseed oil, bleached shellac and absolute alcohol. 90

3. A composition of matter for treating paper to render the same translucent comprising linseed oil, a glazing medium, and a dehydrating agent only.

4. A composition of matter for treating 95 paper to render the same translucent comprising a drying oil, bleached shellac, and a dehydrating agent only.

5. A composition of matter for treating paper to render the same translucent comprising a drying oil, a glazing medium, and absolute alcohol only. 100

6. A composition of matter for treating paper to render the same translucent comprising a drying oil, bleached shellac, and absolute alcohol only. 105

7. In combination, 10 oz. of linseed oil, 3 oz. of bleached shellac and 20 oz. of absolute alcohol.

8. In combination, a drying oil, a dehydrating agent and paper.

In testimony whereof, I affix my signature.

FREDERICK W. HOCHSTETTER.